

# United States Patent

## Goldberg

[15] 3,645,724  
[45] Feb. 29, 1972

### [54] STAINLESS STEEL

[72] Inventor: Robert L. Goldberg, 56 Wilshire Drive, Sharon, Mass. 02067

[22] Filed: Feb. 10, 1969

[21] Appl. No.: 798,120

[52] U.S. Cl. .... 75/126 C, 148/37, 75/126 P

[51] Int. Cl. .... C22c 39/14

[58] Field of Search: 75/126, 126 C, 126 P; 148/37

### [56] References Cited UNITED STATES PATENTS

|           |        |               |          |
|-----------|--------|---------------|----------|
| 2,201,425 | 5/1942 | Berglund..... | 75/126 C |
| 2,590,835 | 4/1952 | Kirkby .....  | 75/126 C |
| 3,250,612 | 5/1966 | Roy .....     | 75/126 P |
| 3,469,972 | 9/1969 | Carlen.....   | 75/126 C |

Primary Examiner—Hyland Bizot  
Attorney—Roberts, Cushman and Grover

### [57]

### ABSTRACT

This invention is for a martensitic, heat hardenable steel of the following composition:

|            |             |
|------------|-------------|
| chromium   | 18 to 20%   |
| molybdenum | 0.2 to 0.8% |
| carbon     | 1.1 to 1.3% |
| boron      | 0 to 0.2%   |
| iron       | balance     |

The alloy is preferably heat tempered at a temperature of from 1,000° to 1,200°F. It is characterized by high wear resistance, corrosion resistance in various media and a freedom from staining. These properties render the steel especially useful for the formation of surgical instruments having a sharp cutting edge.

7 Claims, No Drawings.

## STAINLESS STEEL

## BACKGROUND OF THE INVENTION

## 1. Field of the Invention

This invention relates to martensitic stainless steel and more particularly, to a chromium stainless steel adapted for the formation of surgical instruments requiring a sharp cutting edge.

## 2. Description of the Prior Art

Steels useful for the formation of surgical cutting tools must be characterized by certain properties including high wear resistance which is a function of hardness, corrosion resistance in various media including biological environments and stability and toughness within limits which guarantee an absence of premature staining of the working edge. Chromium stainless steels have been used for the formation of surgical instruments because they are relatively inexpensive, resistant to ordinary corrosive attack, and are capable of being hardened and tempered to desirable strengths.

It is reported in the prior art that heat-treatment affects the corrosion resistance of chromium stainless steels. Heating a hardened steel to temperatures at which carbon precipitates to form chromium carbides is known to be detrimental to overall corrosion resistance because the formation of such carbides robs the steel of the protective action of chromium. For this reason, it has been customary in the prior art to decrease carbon content to improve the corrosion resistance of steels of a given chromium content. However, this is undesirable as it results in a corresponding reduction in hardness.

## DESCRIPTION OF THE INVENTION

The martensitic stainless steel of this invention is an improvement over the stainless steels of the prior art in that both chromium content for corrosion resistance and carbon content for hardness are maintained high. The steel has the following formulation:

|            |             |    |
|------------|-------------|----|
| chromium   | 18 to 20%   | 40 |
| molybdenum | 0.2 to 0.8% |    |
| carbon     | 1.1 to 1.3% |    |
| boron      | 0 to 0.2%   |    |
| iron       | balance     |    |

The above alloy is preferably tempered at a temperature of 45 from 1,000° to 1,200° F. and is characterized by high wear resistance due to hardness, corrosion resistance due to the high

concentration of chromium and stability and toughness within limits which result in an absence of staining. Though not wishing to be bound by theory, it is believed that the high chromium and carbon contents permissible without loss of corrosion resistance is due to the molybdenum and in the preferred embodiment, boron, both of which coreact to induce the formation of martensitic phase.

The invention will be further illustrated by the following examples:

10

## EXAMPLE 1

15

|            |         |
|------------|---------|
| chromium   | 19.5%   |
| carbon     | 1.2%    |
| molybdenum | 0.6%    |
| baron      | 0.1%    |
| iron       | balance |

## EXAMPLE 2

20

|            |         |
|------------|---------|
| chromium   | 20%     |
| carbon     | 1.3%    |
| molybdenum | 0.5%    |
| iron       | balance |

25

The alloys represented in the above two examples are quenched and tempered at a temperature of 1,100° F. followed by slow cooling.

I claim:

1. A martensitic steel consisting essentially of:

30

|            |             |
|------------|-------------|
| chromium   | 18 to 20%   |
| carbon     | 1.1 to 1.3% |
| molybdenum | 0.2 to 0.8% |
| iron       | balance     |

35

2. The composition of claim 1 containing as an additional alloying element up to 0.2 percent boron.

3. The composition of claim 2 where the boron constitutes from 0.1 to 0.2 percent.

4. The steel of claim 1 having the following composition:

40

|            |         |
|------------|---------|
| chromium   | 19.5%   |
| carbon     | 1.2%    |
| molybdenum | 0.5%    |
| iron       | balance |

45

5. The steel of claim 4 containing as an additional alloying element 0.1 percent boron.

6. A surgical tool formed from the steel of claim 1.

\* \* \* \* \*

50

55

60

65

70

75